

## UNITED STATES PATENT OFFICE

2,322,629

## NONFOAMING ASPHALT SATURANT

Henry S. Goodwin, Fanwood, N. J., assignor, by  
mesne assignments, to Standard Catalytic  
Company, a corporation of Delaware

No Drawing. Application February 24, 1941,  
Serial No. 380,311

3 Claims. (Cl. 106—273)

This invention relates to improvements in asphalts employed in saturating materials such as rag felt, asbestos paper, woven fabrics, building boards, etc., and particularly in those asphalts used for such purposes which are solid at ordinary temperatures and are applied in a molten state at elevated temperatures.

In the preparation of asphalt shingles, building boards, and other materials wherein rag felt, asbestos paper, etc., are saturated with asphalt, an elevated temperature of about 400° F. is required. The rag felt or other fibrous material that is used generally contains small amounts of moisture which is difficult to remove without subjecting the material to elevated temperatures for extended periods of time and with attendant loss in the tensile strength of the materials to be treated. On bringing the rag felt containing the small percentages of moisture into contact with the hot asphalt saturant objectionable foaming takes place.

The extent of the foaming is appreciably influenced by the amount of moisture brought into contact with the hot asphalt by the temperature of the asphalt, and by properties of the asphalt

5 It is an object of this invention to prepare an asphaltic material which will not foam excessively and/or will form an unstable (rapidly breaking) foam, when brought into contact with moist materials such as rag felts, etc., at an elevated temperature.

According to this invention the addition of a small amount of sulfonated fatty oil to an asphalt appreciably reduces the stability or tenacity of 10 the foam formed when the heated asphalt and moist materials are brought into contact. I have found that sulfonated animal fats are most suitable and effective, particularly sulfonated tallow.

The asphaltic material that is to be used in 15 saturating the felts, asbestos sheets, etc., employed in the production of asphaltic roofing, building boards, and the like, is first pretreated by the incorporation of small amounts of the sulfonated fats. For example, sulfonated tallow, when introduced into the asphalt in amounts up to 0.20% greatly reduces the tenacity (or lasting quality) of the foam. Pre-treatment of the asphalt in greater amounts than 0.20% of the tallow, on the other hand, causes greater tenacity 20 of the foam as shown in the following table:

*Effect of sulfonated tallow as a foam depressor  
for asphalt saturant*

| Composition of sample         |                    | Physical inspections of blend |                | J. M. research lab. foam test results |                        |                         |
|-------------------------------|--------------------|-------------------------------|----------------|---------------------------------------|------------------------|-------------------------|
| Asphalt used                  | Sulfo-nated tallow | S. P.                         | Pen. at 77° F. | Height of foam rise                   | Time to 1st clear spot | Time to total clearance |
| Venezuelan heavy flux         | Per cent           | °F.                           | Inches         | Inches                                | Secs.                  | Secs.                   |
| Do.                           | 0.00               | 100                           | 170            | 2 <sup>1</sup> / <sub>2</sub>         | 95                     | 460                     |
| Do.                           | 0.05               | 103                           | 160            | 2                                     | 75                     | 360                     |
| Do.                           | 0.10               | 105                           | 163            | 2                                     | 85                     | 380                     |
| Do.                           | 0.20               | 103                           | 166            | 2                                     | 88                     | 465                     |
| Do.                           | 0.40               | 103                           | 167            | 2 <sup>1</sup> / <sub>4</sub>         | 110                    | 1,020                   |
| Do.                           | 0.80               | 102                           | 177            | 2 <sup>1</sup> / <sub>2</sub>         | 1,350                  | 1,850+                  |
| Do.                           | 1.60               | 101                           | 204            | 2 <sup>1</sup> / <sub>2</sub>         | 1,750                  | 1,850+                  |
| Venezuelan roofers' flux      | 0.00               | 106                           | 192            | 2 <sup>1</sup> / <sub>4</sub>         | 245                    | 960                     |
| Do.                           | 0.05               | 106                           | 197            | 2                                     | 205                    | 845                     |
| Do.                           | 0.10               | 105                           | 198            | 2                                     | 195                    | 830                     |
| Do.                           | 0.20               | 105                           | 201            | 2 <sup>3</sup> / <sub>4</sub>         | 190                    | 825                     |
| Do.                           | 0.40               | 105                           | 210            | 2                                     | 185                    | 800                     |
| Colombian heavy flux          | 0.00               | 106                           | 163            | 2                                     | 462                    | 1,100+                  |
| Do.                           | 0.05               | 107                           | 158            | 1 <sup>3</sup> / <sub>4</sub>         | 320                    | 870                     |
| Do.                           | 0.10               | 107                           | 158            | 1 <sup>3</sup> / <sub>4</sub>         | 365                    | 1,090                   |
| Do.                           | 0.20               | 106                           | 154            | 2 <sup>1</sup> / <sub>4</sub>         | 285                    | 1,850+                  |
| Do.                           | 0.40               | 105                           | 151            | 2 <sup>1</sup> / <sub>4</sub>         | 650                    | 1,850+                  |
| Colombian roofers' flux       | 0.00               | 106                           | 179            | 2 <sup>1</sup> / <sub>2</sub>         | 335                    | 1,175                   |
| Do.                           | 0.05               | 104                           | 171            | 2 <sup>1</sup> / <sub>4</sub>         | 240                    | 815                     |
| Do.                           | 0.10               | 105                           | 173            | 2 <sup>3</sup> / <sub>4</sub>         | 245                    | 940                     |
| Do.                           | 0.20               | 106                           | 175            | 2 <sup>3</sup> / <sub>4</sub>         | 210                    | 870                     |
| Do.                           | 0.40               | 106                           | 182            | 2 <sup>1</sup> / <sub>2</sub>         | 510                    | 1,850+                  |
| Venezuelan 100/120 Pen. (ox.) | 0.00               | 114                           | 107            | 2                                     | 190                    | 640                     |
| Do.                           | 0.05               | 115                           | 108            | 1 <sup>3</sup> / <sub>4</sub>         | 155                    | 600                     |
| Do.                           | 0.10               | 115                           | 105            | 2 <sup>1</sup> / <sub>4</sub>         | 128                    | 520                     |

which tend to stabilize the foam that is formed. The foaming characteristics appear to be inherent in the asphalt but may be modified by the addition of suitable quantities of such agents as are indicated herein.

Alternately, the addition to asphalt of small amounts of the sodium sulfonate salts of isobutyl phenol derivatives or lauryl amine modifies the foaming properties of the asphalt so that such 60 asphalt, when caused to foam by contact with

moisture, does not form a stable or slow breaking foam. The salts found most suitable and effective are the sodium sulfonate salts of tetra-isobutyl phenol or of triisobutyl phenol. The sodium sulfonate salt of tetra-isobutyl phenol is preferred. The amount of the salt used may be varied from 0.05 to 0.1% in either case.

The asphalt material that is to be used in the preparation of asphalt shingles, building boards, and other materials is first pretreated by the incorporation of the sodium sulfonate salt of one of the isobutyl phenol derivatives. For example, the sodium sulfonate salt of tetra-isobutyl phenol, when introduced into the asphalt in amounts up to 0.1% greatly reduces the tenacity (or lasting quality) of the foam. Pretreatment in greater amounts than 0.1% of the salt, on the other hand, may cause greater tenacity of the foam.

The following table illustrates the beneficial effects obtained:

*Asphalt used: Colombian 180/200 Pen (ox.) flux*

| Agent used                        | Sodium sulfonate salt of— |                       |                     | 0.05 |
|-----------------------------------|---------------------------|-----------------------|---------------------|------|
|                                   | None                      | Tetra-isobutyl phenol | Tri-isobutyl phenol |      |
| Percent agent added.....          | 0.00                      | 0.05                  | 0.10                | 0.05 |
| <i>Foam test results</i>          |                           |                       |                     |      |
| Height of foam rise.....          | 2½                        | 2½                    | 2¾                  | 3¼   |
| Time to 1st clearance.....seconds | 335                       | 245                   | 285                 | 270  |
| Time to total clearance.....do    | 1,175                     | 920                   | 980                 | 325  |

The additions of small amounts of lauryl amine, 0.02% or more by weight, likewise decreases the foaming action of asphalts.

The following experimental laboratory data illustrate the advantage of using lauryl amine as a foam depressant:

**I. ASPHALT FLUX EMPLOYED: 156° S. P. OXIDIZED VENEZUELAN SHINGLE SATURANT**

| Lauryl amine added | Softening point | Pen. 77° F. | Height of foam | Retention time of foam |
|--------------------|-----------------|-------------|----------------|------------------------|
| Per cent           | °F.             |             | Inches         | Seconds                |
| None               | 156             | 30          | 5½             | 85                     |
| 0.04               | 152             | 30          | 5½             | 55                     |

(These blends prepared at 300-350° F.)

**II. ASPHALT FLUX EMPLOYED: COLOMBIAN ROOFERS' FLUX**

| Lauryl amine added | Softening point | Pen. 77° F. | Retention time of foam |
|--------------------|-----------------|-------------|------------------------|
| Per cent           | °F.             |             | Seconds                |
| None               | 102             | 179         | 430                    |
| 0.1                | 105             | 180         | 410                    |
| 0.2                | 104             | 182         | 420                    |
| 0.4                | 104             | 187         | 370                    |
| 1.2                | 103             | 227         | 385                    |

(These blends prepared at 300-350° F.)

**III. ASPHALT FLUX EMPLOYED: COLOMBIAN ROOFERS' FLUX**

| Lauryl amine added | Softening point | Pen. 77° F. | Retention time of foam |
|--------------------|-----------------|-------------|------------------------|
| Per cent           | °F.             |             | Seconds                |
| None               | 105             | 172         | 605                    |
| 0.2                | 105             | 178         | 575                    |
| 0.4                | 106             | 187         | 490                    |
| 1.0                | 103             | 217         | 480                    |

(These blends prepared at 250-300° F.)

15 The above data indicate that the maximum foam reduction appears to have been obtained by the addition of 0.4% (or more) of the lauryl amine.

Lauryl amine might also be employed as a foam depressant for other materials such as transformer oils, lubricating oils, quenching oils, etc.

20 The foaming of the asphalts according to the above tables were compared by the following method.

25 Two hundred grams of the asphalt under test are heated to 420° F. and 185 grams of this are poured into a thin walled cylindrical copper container open at the top, having an inside diameter of 4½ inches and 11 inches high, with small lugs placed 1½, 2½, 3½, 5, 6, 7, 8, 9 and 10 inches from the bottom. The container is well lagged on the sides but not on the bottom. The asphalt and container is maintained at a temperature of 400° F. plus or minus 3° F. A sheet of blotting paper, 3 x 3 inches in area, is air dried and moistened with 3.3 ml. of water in such a manner than even saturation of the paper is obtained in approximately 45 seconds. The wet paper is immersed in the hot asphalt and pushed to the bottom of the container with a stirring rod. Observations are made of the maximum height to which the foam rises, and the period of time from the introduction of the water-moistened paper until the foam has subsided to the lug placed 2½ inches from the bottom of the container, this being the subsidence time. As the foam subsides the stirring rod is gently run around the edge of the foam in order to promote even subsidence, and to more closely detect the time at which the foam reaches the 2½ inch lug.

50 I claim:

1. An asphalt saturant for fibrous material comprising a mixture of 99.8 to 99.95% of an asphalt and 0.20% to 0.05% of sulfonated tallow.

2. An asphalt saturant for fibrous material comprising a mixture of an asphalt and not over 0.20% of sulfonated tallow.

3. In the saturating of fibrous material, the 55 step which comprises adding to a foamable fibrous material a mixture consisting of 0.20. to 0.05% of sulfonated tallow to 99.8 to 95.8% of asphalt.

HENRY S. GOODWIN.